

# UNITED STATES PATENT OFFICE.

HARRY L. HAAS, OF NEW YORK, N. Y.

## POLISHING COMPOUND.

SPECIFICATION forming part of Letters Patent No. 244,595, dated July 19, 1881.

Application filed June 8, 1881. (No specimens.)

*To all whom it may concern:*

Be it known that I, HARRY L. HAAS, of the city of New York, in the county and State of New York, have invented a new and Improved 5 Polishing Compound, of which the following is a specification.

This invention relates to polishing compounds to be used for preparing buff-wheels or polishing-buffs or other devices or surfaces 10 employed for the polishing of metal and other substances. Such compounds are ordinarily made of rouge, crocus, tripoli, emery, corundum, lime, or other mineral powder, or a mixture of two or more such powders, and a certain 15 proportion of stearine, paraffine, or other binding material, which will hold the grains of the powder together in the form of a cake or stick. The stearine or binding material has no polishing quality, but rather impairs the 20 polishing quality of the mineral powder, and is only used in the compound in the smallest quantity that suffices to hold the powder to the wheels or buffs or other polishing-surfaces to which the compound is applied by pressing 25 the cake or stick against them while they are in motion.

In making experiments with various binding materials for the manufacture of polishing compounds of the character hereinabove mentioned, 30 I have discovered that ozocerite possesses the qualities necessary to such binding material in a very marked degree—that is to say, first, its binding quality is greater than that of stearine, paraffine, or the binding materials heretofore employed, so that a smaller 35 quantity of it in proportion to the quantity of the powder is sufficient, and the cakes or sticks are not so liable to break or crumble when pressed against the wheels or buffs; second, 40 as it is not of a greasy nature it does not impair the polishing quality of the powder, but,

on the contrary, its peculiar waxy nature rather improves the said quality; third, it holds the compound better to the wheels or buffs when the latter are in rapid motion, so that it will 45 not fly off; fourth, it is cheaper than the stearine or paraffine.

The quantity of the ozocerite which I use in the compound in proportion to the polishing mineral powder may be varied considerably, but may generally be from ten (10) pounds to twenty-five (25) pounds of ozocerite to one hundred (100) pounds of the powder, consisting of rouge, crocus, tripoli, emery, corundum, lime, or other mineral substance commonly 50 used or suitable for polishing purposes, or a mixture of two or more such substances, a greater proportion being generally necessary for the finer grades and a smaller proportion for the coarser grades of polishing substance. 55

To make the compound the ozocerite is melted in a suitable vessel heated by a fire or by other suitable means, and while this is kept at melting-heat the mineral powder is added to it and stirred and worked or rubbed 60 into it until thoroughly incorporated, and while the compound is still plastic it is molded or pressed, or otherwise formed into sticks or slabs of suitable or convenient size for use. 65

Various kinds of ozocerite may be used, 70 either crude or purified; but the crude, being cheaper, and making as good a compound as the purified, is preferable.

What I claim as my invention, and desire to secure by Letters Patent, is—

A polishing compound consisting of a mineral polishing-powder and ozocerite, substantially as herein described.

H. L. HAAS.

Witnesses:

HENRY T. BROWN,  
FREDK. HAYNES.